

## UNITED STATES PATENT OFFICE

2,382,144

## GELATINATION OF HYDROCARBON DISTILLATES

William K. Griesinger, Drexel Hill, Pa., assignor to  
 The Atlantic Refining Company, Philadelphia,  
 Pa., a corporation of Pennsylvania

No Drawing. Application August 25, 1943,  
 Serial No. 500,187

8 Claims. (Cl. 44—7)

This invention relates to the gelatination or congelation of hydrocarbon distillates to produce solidified fuels suitable for use in incendiaries and for heating purposes and the like.

The production of solidified fuels from normally liquid hydrocarbon distillates by the incorporation therewith of fatty acid soaps such as sodium stearate has previously been disclosed. I have now found that solidified fuels of superior characteristics may be prepared from hydrocarbon distillates by means of a gelling agent consisting of a solution of alkali sulfonates and a basic material in water.

The alkali sulfonates employed in the preparation of my gelling agent or solution are distinguished from other alkali sulfonates in that they are relatively more soluble in water than in hydrocarbon oil. They may be produced through the neutralization of sulfonic acids extractable, as with benzol, from the separable sludge which develops when various hydrocarbon oils such as cracked petroleum distillates, coal tar distillates, etc., are subjected to treatment with fuming sulfuric acid or other sulfonating agent to remove undesirable constituents.

Normally liquid hydrocarbon distillates which may be solidified according to the invention include petroleum fractions such as naphtha, gasoline, benzine, kerosene, furnace oil, fuel oil, etc., the lighter fractions, particularly gasoline, being preferred. Since by my process I may effect the solidification of individual hydrocarbons as well as hydrocarbon fractions, the term "hydrocarbon distillates" as used herein and in the appended claims is intended as encompassing both individual hydrocarbons and hydrocarbon fractions.

The basic material in my gelling agent is most suitably an alkali metal hydroxide such as sodium hydroxide or potassium hydroxide, but other alkaline compounds, such as borax, sodium carbonate, potassium carbonate, and di- or tri-sodium phosphate may be employed if desired.

Although my gelling agent may be made up to contain only a single alkali sulfonate, it is my practice to utilize the sulfonates mentioned above obtained by the neutralization of sulfonic acids extracted from acid sludges, and these are available only in mixtures from which it would be commercially impractical to attempt the separation of an individual sulfonate. I especially prefer petroleum sulfonates, i. e., sulfonates derived from petroleum acid sludge.

In the preparation of the gelling agent, the sulfonates may be dissolved in the water, and

the basic material thereafter added, or the basic material may be first dissolved in the water. If desired, instead of sulfonates, I may use sulfonic acids during the preparation of the solution as these would be immediately saponified by the alkali to give the sulfonates. Where this practice is followed, it is essential to use an excess of the alkali over and above the amount required to effect the conversion, otherwise a stable gel will not result when the solution is subsequently used to effect the solidification of a hydrocarbon distillate.

Although I have obtained excellent results with a solution which contained 20 weight per cent sulfonates and 10 weight per cent basic material, these proportions are not critical. I consider the permissible limits to be as follows:

|                | Per cent by weight |
|----------------|--------------------|
| Water          | 60 to 45           |
| Sulfonates     | 10 to 40           |
| Basic material | 5 to 15            |

The solidification of hydrocarbon distillates by means of the herein described gelling agent is effected by intimately mixing the gelling agent with the hydrocarbon distillate it is desired to solidify. The mixing may be carried out in any suitable type of apparatus at ordinary temperature. The amount of gelling agent used may vary from 0.5 to 10 per cent of the volume of the distillate.

My invention is further illustrated by the following example which is not, of course, to be taken as limiting the scope thereof: 98 volumes of gasoline was thoroughly admixed with 2 volumes of an aqueous solution containing 20 per cent by weight of water-soluble petroleum sulfonates and 10 per cent by weight of sodium hydroxide, the mixing being accomplished by shaking the gasoline and aqueous solution at room temperature. The resulting product was a gel stable at temperatures up to 130° F. The petroleum sulfonates used in the preparation of the gelling solution were derived from an acid sludge separated from a partially cracked gas oil fraction which had been treated with sulfuric acid.

The solidified hydrocarbon distillates produced in accordance with the invention are adapted for a variety of uses. They may, for example, be burned in the open or in a container or stove to provide heat as for cooking, or may be used in lieu of liquid fuels in cigarette lighters and the like. In wartime they may be employed in the manufacture of incendiary bombs, being well adapted for this purpose.

I claim:

1. A process for producing a solidified fuel from a hydrocarbon distillate without the aid of a fatty acid soap which comprises mixing the distillate with from 0.5 per cent to 10 per cent by volume of an aqueous solution of water-soluble alkali metal petroleum sulfonates and an alkali metal hydroxide, said solution containing from 10 to 40 per cent by weight of petroleum sulfonates, and from 5 to 15 per cent by weight of the alkali metal hydroxide.

2. A process for producing a solidified fuel which comprises agitating 98 parts by volume of a hydrocarbon distillate with two parts by volume of an aqueous solution containing 20 per cent by weight of water-soluble alkali metal petroleum sulfonates and 10 per cent by weight of sodium hydroxide.

3. A process for producing a solidified fuel which comprises agitating 98 parts by volume of gasoline with 2 parts by volume of an aqueous solution containing 20 per cent by weight of water-soluble alkali metal petroleum sulfonates and 10 per cent by weight of sodium hydroxide, said petroleum sulfonates having been obtained by the neutralization of sulfonic acids derived from an acid sludge produced by the treatment of a partially cracked gas oil fraction with a sulfonating agent.

4. A solidified fuel comprising a hydrocarbon distillate and from 0.5 to 10 per cent by volume of a gelling agent containing from 10 to 40 per cent by weight of water-soluble alkali metal petroleum sulfonates, 5 to 15 per cent by weight of sodium hydroxide, and 45 to 65 per cent by weight

of water, said solidified fuel being free of fatty acid soaps.

5. A solidified fuel comprising 98 parts by volume of gasoline and about 2 parts by volume of a gelling agent containing 20 per cent by weight of water-soluble alkali metal petroleum sulfonates, 10 per cent by weight of sodium hydroxide, and 70 per cent by weight of water.

10 6. A process for producing a solidified fuel from a hydrocarbon distillate without the aid of a fatty acid soap which comprises mixing the distillate with from 0.5 per cent to 10 per cent by volume of an aqueous solution of water-soluble alkali metal hydrocarbon sulfonates and an alkali metal hydroxide, said solution containing from 15 10 to 40 per cent by weight of hydrocarbon sulfonates, and from 5 to 15 per cent by weight of the alkali metal hydroxide.

20 7. A process for producing a solidified fuel which comprises agitating 98 parts by volume of a hydrocarbon distillate with two parts by volume of an aqueous solution containing 20 percent by weight of water-soluble alkali metal hydrocarbon sulfonates and 10 per cent by weight 25 of sodium hydroxide.

8. A solidified fuel comprising a hydrocarbon distillate and from 0.5 to 10 per cent by volume of a gelling agent containing from 10 to 40 per cent by weight of water-soluble alkali metal hydrocarbon sulfonates, 5 to 15 per cent by weight of sodium hydroxide, and 45 to 65 per cent by weight of water, said solidified fuel being free 30 of fatty acid soaps.

35

WILLIAM K. GRIESINGER.

CERTIFICATE OF CORRECTION.

Patent No. 2,382,144.

August 14, 1945.

WILLIAM K. GRIESINGER.

It is hereby certified that error appears in the printed specification of the above numbered patent requiring correction as follows: Page 1, second column, line 19, for "60 to 45" read --65 to 45--; and that the said Letters Patent should be read with this correction therein that the same may conform to the record of the case in the Patent Office.

Signed and sealed this 4th day of December, A. D. 1945.

Leslie Frazer

(Seal)

First Assistant Commissioner of Patents.